

## UNITED STATES PATENT OFFICE

RAYMOND I. BASHFORD, OF PHILADELPHIA, PENNSYLVANIA, ASSIGNOR, BY MESNE ASSIGNMENTS, TO ATLAS POWDER COMPANY, A CORPORATION OF DELAWARE

## LOW DENSITY EXPLOSIVE

No Drawing.

Application filed January 23, 1932. Serial No. 588,503.

My invention relates to a low density dynamite and material for use in conjunction therewith, and more particularly it relates to explosives of the ammonium nitrate type suitable for mining coal in gaseous mines.

One object of my invention is to provide an explosive of the permissible type containing ammonium nitrate, which explosive is relatively bulky, but at the same time highly sensitive.

A further object is to furnish an ammonium nitrate explosive, suitable for mining coal in gaseous mines in which a portion of the dense sodium nitrate is replaced by a relatively bulky, light, inert material.

Another object is to produce a material for use in ammonium nitrate explosives which is of low density and occupies a relatively large space and which may be added to the explosive without reducing its sensitivity and without requiring oxygen during the explosion or detonation.

Still another object is to provide a method of treating inert material to render it suitable for use in ammonium nitrate explosives in conjunction with nitro-glycerine.

Other objects will be apparent from a consideration of the specification and claims.

The bulky ammonium nitrate low density explosives are to be desired in many instances, since there are more sticks per unit of weight and the explosive is distributed over a larger area in the bore hole than is the case with the standard explosives. Heretofore difficulty has been encountered in making explosives of the bulky type of low strength, since in these explosives it has been found necessary to reduce the bulk as the strength is lowered. In the explosives of the present invention it is possible to lower the strength of the explosive without appreciably decreasing the bulk or in any way affecting the sensitivity thereof.

One group of the explosives of the present invention has characteristics which satisfy the tests of the Bureau of Mines relating to

the so-called "permissible explosives", and, therefore, it falls within that classification.

My invention contemplates the use of relatively bulky treated inert material to replace a portion of the sodium nitrate which not only is dense, but also requires additional amounts of carbonaceous material to satisfy its oxygen content. The inert material is treated to render it substantially non-absorptive toward nitro-glycerine, and, therefore, it is possible by its use to produce an explosive whose sensitiveness is not decreased. The inert material may be infusorial earth, known variously as kieselguhr, diatomaceous earth, fossil flour, etc., or finely divided or shredded asbestos, bulky in nature and light in weight, or like materials which will not require oxygen in the explosion or detonation. The inert material prior to its mixture in the explosive compound is treated by bringing it in contact with a solution, preferably one that is saturated, of one or more salts which may or may not function in the explosion, but which do not render the explosive insensitive. Preferably, the oxygen-bearing salts, capable of liberating oxygen during the explosion, are used in the explosive. Since the fumes which prevail upon explosion are such as will allow the explosive to pass the "permissibility test", sodium chloride is an example of a non-oxygen-bearing salt which may be employed without rendering the explosive insensitive. The inert material absorbs the salt until the pores are substantially filled. Hence, the absorptive capacity is reduced to a point where no appreciable nitro-glycerine will be absorbed when it is brought in contact with the treated material.

The inert material may be treated by mixing it with an approximately saturated solution of the salt, for example, sodium nitrate or ammonium nitrate, or a mixture of these oxygen-bearing salts, and allowing it to remain in contact therewith until practically complete absorption has taken place. The

material is then dried and screened free from lumps and is ready for compounding with the other materials which are to be used in making up the explosive. The amount of 5 salt absorbed by the inert material varies widely, and depends upon the nature and condition of the inert material. The treated inert material, for example, may have absorbed salt to an extent where the treated 10 material comprises 20% to 70% inert material and 80% to 30% salt. The particular inert material being treated should have its absorptive capacity substantially satisfied by the salt, so that when it is brought in contact 15 with the nitro-glycerine, it will take practically none of the compound into its pores.

The treated inert material when it contains an oxygen-bearing salt, as hereinbefore pointed out, is successful for use in conjunction 20 with ammonium nitrate explosives of the permissible type. These explosives contain nitro-glycerine and sufficient carbonaceous material to satisfy the oxygen liberated from the 25 oxygen-bearing salt during the explosion or detonation. The explosives usually also contain sodium nitrate and an antacid, and they may or may not contain nitro-cotton.

As typical of the explosives which may be 30 used, the following example is given:

|                                                                                                  | Per cent |
|--------------------------------------------------------------------------------------------------|----------|
| Ammonium nitrate                                                                                 | 30-75    |
| Nitro-glycerine                                                                                  | 9-20     |
| Sodium nitrate                                                                                   | 10-35    |
| Carbonaceous material<br>(wood pulp, etc.)                                                       | 6-17     |
| Antacid (calcium carbonate-zinc<br>oxide, etc.)                                                  | 0-2      |
| Nitro-cotton                                                                                     | 0-1.5    |
| Treated inert material containing<br>from 20% to 70% of inert material<br>and 80% to 30% of salt | 4-25     |
| Nitro-body (tri-nitro-toluene di-nitro-<br>toluene)                                              | 0-15     |

It is to be understood that the limits given are only approximate, and that other substances may be used in place of those given, and other materials may be employed in addition, for example, if desired, salt (sodium chloride) 50 may be added as a flame-reducing agent.

As illustrations, the following formulae have proved to be especially successful, the first of which is compounded without nitro-cotton, while the second one is a nitro-cotton 55 containing explosive:

#### Explosive without nitro-cotton

|                                                                                             | Per cent |
|---------------------------------------------------------------------------------------------|----------|
| Nitro-glycerine                                                                             | 12       |
| Ammonium nitrate                                                                            | 40       |
| Sodium nitrate                                                                              | 12.5     |
| Carbonaceous material                                                                       | 14       |
| Treated infusorial earth containing<br>25% of infusorial earth and 75% of<br>sodium nitrate | 20.5     |
| Antacid (calcium carbonate)                                                                 | 1        |

| Explosive with nitro-cotton                                                                 |            |
|---------------------------------------------------------------------------------------------|------------|
|                                                                                             | Per cent   |
| Nitro-glycerine                                                                             | 17         |
| Ammonium nitrate                                                                            | 42         |
| Sodium nitrate                                                                              | 22         |
| Di-nitro-toluene                                                                            | 1          |
| Nitro-cotton                                                                                | .25        |
| Carbonaceous material                                                                       | 7.5        |
| Antacid (calcium carbonate)                                                                 | 1          |
| Treated fine divided bulky asbestos<br>containing 60% asbestos and 40% of<br>sodium nitrate | 75<br>9.25 |

The explosive of the present invention is a relatively bulky ammonium nitrate explosive low density which is highly sensitive, due to the fact that there is placed in the explosive a bulky inert material which is non-absorptive toward the nitro-glycerine. 80

Considerable modification is possible in the choice of ingredients used in the formula, 85 as well as in the proportions employed, without departing from the essential features of the invention.

I claim:

1. An ammonium nitrate low density explosive having therein a relatively bulky inert material, the pores of which are substantially filled with a salt. 90

2. An ammonium nitrate low density explosive having therein infusorial earth, the pores of which are substantially filled with a salt. 95

3. An ammonium nitrate low density explosive having therein finely divided relatively bulky asbestos, the pores of which are 100 substantially filled with a salt.

4. An ammonium nitrate low density explosive having therein a relatively bulky inert material, the pores of which are substantially filled with an oxygen bearing salt capable of liberating its oxygen during the 105 explosion.

5. An ammonium nitrate low density explosive having therein infusorial earth, the pores of which are substantially filled with an oxygen bearing salt capable of liberating its oxygen during the 110 explosion.

6. An ammonium nitrate low density explosive having therein finely divided relatively bulky asbestos, the pores of which are 115 substantially filled with an oxygen bearing salt capable of liberating its oxygen during the explosion.

7. An ammonium nitrate low density explosive having therein a relatively bulky inert material, the pores of which are substantially filled with sodium nitrate. 120

8. An ammonium nitrate low density explosive comprising ammonium nitrate, nitro-glycerine, sodium nitrate, carbonaceous material sufficient to satisfy the oxygen liberated from the oxygen bearing salts during the explosion, and relatively bulky inert material, the pores of which are substantially filled with an oxygen bearing salt capable 125 130

- of liberating its oxygen during the explosion.
9. An ammonium low density explosive comprising ammonium nitrate, nitro-glycerine, sodium nitrate, carbonaceous material sufficient to satisfy the oxygen liberated from the oxygen bearing salts during the explosion, and infusorial earth, the pores of which are substantially filled with an oxygen bearing salt capable of liberating its oxygen during the explosion.
10. An ammonium nitrate low density explosive, comprising ammonium nitrate, nitro-glycerine, sodium nitrate, carbonaceous material sufficient to satisfy the oxygen liberated from the oxygen bearing salts during the explosion, and relatively bulky finely divided asbestos, the pores of which are substantially filled with an oxygen bearing salt capable of liberating its oxygen during the explosion.
11. An ammonium nitrate low density explosive comprising nitro-glycerine between 9 per cent and 20 per cent; carbonaceous material between 6 per cent and 17 per cent; antacid between 0 per cent and 2 per cent; nitrocotton between 0 per cent and 1.5 per cent; nitro-body between 0 per cent and 15 per cent; treated inert material between 4 per cent and 25 per cent, said inert material containing between 20 per cent and 70 per cent of inert material and 80 per cent and 30 per cent of oxygen bearing salt capable of liberating oxygen during the explosion; ammonium nitrate between 30 per cent and 75 per cent; and sodium nitrate between 10 per cent and 35 per cent, the amounts of the two latter ingredients being independent of the amount of oxygen bearing salt carried by the inert material, the explosive being made up of the said ingredients to total 100 per cent.
12. An ammonium nitrate low density explosive comprising nitroglycerine approximately 12 per cent, carbonaceous material approximately 14 per cent, antacid approximately 1 per cent, treated inert material approximately 20.5 per cent, said inert material containing approximately 25 per cent of infusorial earth and 75 per cent of sodium nitrate; ammonium nitrate approximately 40 per cent and sodium nitrate approximately 12.5 per cent, the amount of sodium nitrate being independent of the amount of sodium nitrate carried by the inert material; the explosive being made up of the said ingredients to total 100 per cent.
13. An ammonium nitrate low density explosive comprising nitroglycerine approximately 17 per cent, carbonaceous material approximately 7.5 per cent, antacid approximately 1 per cent, treated inert material approximately 9.25 per cent, said inert material containing approximately 60 per cent of finely divided bulky asbestos and 40 per cent of sodium nitrate; ammonium nitrate approximately 42 per cent, dinitrotoluene ap-
- proximately 1 per cent, nitrocotton approximately .25 per cent, and sodium nitrate approximately 22 per cent, the amount of sodium nitrate being independent of the amount of sodium nitrate carried by the inert material; the explosive being made up of the said ingredients to total 100 per cent.
- RAYMOND I. BASHFORD.
- 70
- 75
- 80
- 85
- 90
- 95
- 100
- 105
- 110
- 115
- 120
- 125
- 130